

Patented May 2, 1950

2,506,309

## UNITED STATES PATENT OFFICE

2,506,309

## COMPOSITION HAT PRESSING BLOCK

George Middleman, Brooklyn, N. Y.

No Drawing. Application December 17, 1946,  
Serial No. 716,879

2 Claims. (Cl. 260—17.3) ✓

1

This invention relates to a composition hat pressing block. While not limited thereto, it is more particularly concerned with a composition block for pressing, especially useful for the pressing of hats by hand or machine, and to a method for preparing the same.

Using the new invention, it is possible to make a pressing block which will not normally burn and which will thus readily withstand the abuses of unskilled pressing, negligence or delay in pressing operations.

Moreover, the new product will readily form in any customary mold, using nothing but simple pouring and relatively short curing cycle. Once finished, no trimming will be necessary for the product except in the case of the first model.

The product of the new invention and its process of manufacture can thus be handled with ease and substantially without difficulty, in spite of and in addition to all the above enumerated advantages and to many others which will readily occur to those skilled in the art reading the instant specification.

Moreover, the new invention contemplates a product made from economical and readily available materials and one which can be made practically, using inexpensive readily available machinery and standard, or simplified standard, manufacturing steps.

Ornaments and other decorative or simplified changes in the form may readily be made in the product of the invention.

For further comprehension of the invention, and of the objects and advantages thereof, reference will be had to the following description, and to the appended claims in which the various novel features of the invention are more particularly set forth.

In accordance with the invention, a pressing form is made using as body a balanced finely divided fibrous filler suspended in a composition composed of an inert mineral filler and a combination of a mineral agglutinant binder of high binding power and an organic agglutinant of high binding power.

The preferred fibrous filler is balanced as to elastic and fibrous compression quality such as wood in the form of sawdust, finely shredded cloth, paper, or sisal. These materials should all be finely divided and have the common property of fibrous resistance against undue sudden compression together with a slight degree of inherent recovery, elasticity and easy blending into binders.

The inert mineral filler should be of the class

2

consisting of plaster of Paris, again finely divided, and its equivalents. This product will easily blend with the sawdust due to their cooperating elasticity-rigidity functions.

5 The mineral agglutinant will be of the class comprising the sodium and potassium silicates. A suitable grade of sodium silicate for instance is available under the name Grade N. The silicate has extremely high binding powder and 10 some fibrous impregnation-penetration properties which cooperate to completely bind the fibrous filler.

To make the silicate more elastic and cooperative in its binding action, an organic high binding power agglutinant such as glue or viscous polyvinyl alcohol will be added. The two agglutinants combine very thoroughly and secure binding action for the filler with elastic shock resistant properties, which provides for long wear and continued reuse of the product of the invention.

It is preferable to prepare the product so that the finished product is approximately in the following parts by volume per part of inorganic agglutinant binder:

1/5 parts of organic agglutinant binder  
2/8 parts of inorganic mineral filler  
7/15 parts of finely divided fibrous filler

30 In a preferred example the following proportions will be present:

## Example

|                                      | Cups |
|--------------------------------------|------|
| Sodium silicate (20% solution) ----- | 5    |
| 35 Plaster of Paris -----            | 5    |
| "Casco Resin" glue -----             | 2½   |
| Sawdust -----                        | 10   |

Instead of the "Casco Resin," which is a liquid 40 urea-formaldehyde resin glue, in the above example, melamine aldehyde or ordinary glue may be used.

In a preferred execution of the method, the finely divided plaster of Paris and sawdust are first mixed. In a separate container, a dilute solution of glue is combined with the sodium silicate solutions under constant stirring and slight heating. The first mixture is then slowly added there-to.

50 Mixing and stirring should be continued until a putty like consistency is obtained. The mass is then poured into a mold and dried in a hot oven. It should then stand for approximately two hours. It may be then corrected or carved to a desired shape.

This composition may also be used for any other useful purpose in addition to its use for hat pressing blocks and it may be sold in block forms or sheets.

While I have described the preferred embodiments of my invention, it is to be understood that I do not limit myself to the precise constructions herein disclosed and the right is reserved to all changes and modifications coming within the scope of the invention as defined in the appended claims.

Having thus described my invention, what I claim as new, and desire to secure by United States Letters Patent is:

1. A pressing block composed of five cups of plaster of Paris, ten cups of sawdust from wood, five cups of sodium silicate, and two and one-half cups of liquid urea-formaldehyde resin glue to make the sodium silicate more elastic.

2. The method of making a pressing block, which consists in dry mixing five cups of plaster of Paris and ten cups of sawdust from wood, separately mixing five cups of sodium silicate

and two and one-half cups of liquid urea-formaldehyde resin glue, combining the two mixtures, stirring the resulting mass until a putty-like consistency is obtained, pouring the mass in a mold, drying the mass in a hot oven, allowing the dried mass to stand for two hours, and shaping and carving the mass to a desired shape.

GEORGE MIDDLEMAN.

#### REFERENCES CITED

The following references are of record in the file of this patent:

#### UNITED STATES PATENTS

| Number    | Name     | Date          |
|-----------|----------|---------------|
| 83,495    | Hathaway | Oct. 27, 1868 |
| 1,667,019 | Venzie   | Apr. 24, 1908 |
| 1,988,242 | Gugger   | Jan. 15, 1935 |
| 2,132,782 | Fernbach | Oct. 11, 1938 |

#### FOREIGN PATENTS

| Number | Country       | Date    |
|--------|---------------|---------|
| 11,522 | Great Britain | of 1908 |